

April 3, 1973

A. B. KUPER  
OXIDATION OF SEMICONDUCTIVE ALLOYS  
AND PRODUCTS OBTAINED THEREBY

3,725,161

Filed March 3, 1971

6 Sheets-Sheet 1



INVENTOR  
ALAN B. KUPER

Fig. 4  
McNenny, Farrington, Pearne & Gordon  
ATTORNEYS

April 3, 1973

A. B. KUPER  
OXIDATION OF SEMICONDUCTIVE ALLOYS  
AND PRODUCTS OBTAINED THEREBY

3,725,161

Filed March 3, 1971

6 Sheets-Sheet 2



INVENTOR  
ALAN B. KUPER

McNenny, Farrington, Pearne & Gordon  
ATTORNEYS

April 3, 1973

Filed March 3, 1971

**A. B. KUPER**  
OXIDATION OF SEMICONDUCTIVE ALLOYS  
AND PRODUCTS OBTAINED THEREBY

3,725,161

6 Sheets-Sheet 3



INVENTOR  
ALAN B. KUPER

McNenny, Farrington, Pearne & Gordon  
ATTORNEYS

April 3, 1973

**A. B. KUPER**  
**OXIDATION OF SEMICONDUCTIVE ALLOYS**  
**AND PRODUCTS OBTAINED THEREBY**

3,725,161

Filed March 3, 1971

6 Sheets-Sheet 4



INVENTOR  
ALAN B. KUPER

*McNenny, Farrington, Pearne & Gordon*  
**ATTORNEYS**

April 3, 1973

Filed March 3, 1971

A. B. KUPER  
OXIDATION OF SEMICONDUCTIVE ALLOYS  
AND PRODUCTS OBTAINED THEREBY

3,725,161

6 Sheets-Sheet 5



INVENTOR  
ALAN B. KUPER

McNally, Farrington, Pearce & Gordon  
ATTORNEYS

April 3, 1973

A. B. KUPER  
OXIDATION OF SEMICONDUCTIVE ALLOYS  
AND PRODUCTS OBTAINED THEREBY

3,725,161

Filed March 3, 1971

6 Sheets-Sheet 6



FIG. 13



FIG. 14

INVENTOR  
ALAN B. KUPER

McNenny, Farrington, Pearne & Gordon  
ATTORNEYS

**1**

3,725,161

**OXIDATION OF SEMICONDUCTIVE ALLOYS AND PRODUCTS OBTAINED THEREBY**Alan B. Kuper, 2265 Delaware Drive,  
Cleveland Heights, Ohio 44106Filed Mar. 3, 1971, Ser. No. 120,448  
Int. Cl. B44d 5/12; H01L 11/00

U.S. CL. 156—17

14 Claims

**ABSTRACT OF THE DISCLOSURE**

There is provided a process for producing from certain semiconductive alloys, e.g. an alloy of silicon and germanium, with or without dopants, a composite body having an oxidized coating on a bulk body of the alloy, and in which there is an increased concentration of one of the elements, e.g. germanium, at the interface and in the subsurface and whereby the oxide composition is controlled and wherein the bulk body of the alloy is subjected to a predetermined number of operational cycles from 1 to 10 or more, each cycle including oxidation, e.g. thermal oxidation, in a chemically oxidizing environment, e.g. an oxygen-containing or yielding gaseous medium. Following oxidation, etching of the oxide coating may optionally be performed, or an oxidation/etching cycle repeated. Novel semiconductor materials are obtained by this process which afford advantages in fabrication and performance of devices.

**BACKGROUND OF THE INVENTION**

The present invention concerns the oxidation of alloys, usually single crystals, of at least two principal component elements and products obtained thereby. Principal among such alloys are those binary systems of silicon and germanium, which will be used for illustrative purposes herein. The principal components of the alloys or compositions of elements in accordance herewith are present in significant amounts, preferably at least about 1.0 atom percent, and are to be distinguished in kind from trace donor or acceptor impurities called "dopants" such as in the case of Si, which may be "doped" with other elements, e.g. P, B, Al, Sb or the like, in trace amounts measured in parts per million and usually not exceeding about 500 p.p.m. As indicated below, dopants may be present in these compositions in the trace amounts usually employed for such materials, but in any event at least two principal component elements are also present.

A principal alloying constituent, such as Ge in SiGe alloy, is to be distinguished fundamentally from a doping impurity not only in that its concentration is significantly larger but that (1) Ge is a group IV element and does not dope Si, (2) Ge is an integral part of the SiGe alloy such that all parameters of the system are affected in a major way by its presence, in contrast to the effect on Si of a dopant, which is principally to change electrical conductivity.

Germanium and silicon are Group IV elements, similar in many respects except in respect to their relative oxidizability, i.e. they are differentially oxidizable. Both are important commercial semiconductors usually used as single crystals. They form a continuous series of solid solutions when crystals are made from a mixture of the two elements. Solid Ge and Si differ in band structure, chemical activity with regard to impurities, and in many other related ways. These differences lead to different technologies for the two, with different advantages in fabrication and use.

In semiconductor technology composite bodies comprising a silicon base, possibly doped, and a silicon oxide coat are currently used. A typical example of such a use is a P-type silicon base having selectively diffused

**2**

therein a plurality of units comprising each two N-type regions separated from each other and serving as source and drain, a silicon oxide coat spanning the gap between said N-type regions, and an electrode, e.g. of aluminum, applied to the silicon oxide layer. Each such unit serves as a triode and the performance thereof depends on the characteristics of the system. These in turn are dependent on the characteristics of the oxide coat, of the oxide-bulk interface, and of the bulk layer below the interface.

5 For example, the offset voltage and the triode transconductance depend principally on the nature of the oxide and interface, respectively. The conductivity between source and drain with the device conducting (and also the energy gap and band structure) depend principally on

10 15 the composition of the subsurface alloy.

In general, the properties of the oxide coat are important in fabrication and performance of a semiconductor device. Among such properties there may be mentioned the permeability to impurities, built-in charge relative to semiconductor surface, dielectric constant, growth-rate and etch-rate, dielectric strength, conductance, optical properties, glass-forming properties, mechanical properties and thermal properties.

It may be stated quite generally that the performance 25 of every semiconductor device comprising a semiconductor body coated with an oxide layer is the resultant of an interplay between the properties of the oxide, the nature of the oxide-bulk interface, and the properties of the bulk layer immediately below said interface. It has now

30 35 40 45 50 55 60 65 70

been found that by modifying the properties of these three components in a novel controlled manner, the performance of a semiconductor may be influenced in a desired way.

Where an oxide coat is grown on a substrate consisting 35 of an alloy of elements, the properties of the oxide-bulk interface or of the bulk surface are as a rule different from the properties of the bulk and of the clean, etched surface prior to any oxidation. Where the substrate is a semiconductor, the performance of the body depends 40 to an important degree on the nature of the surface and oxide, the oxide-bulk interface, and also depends on the bulk layer immediately below that surface. Hereinafter the combined properties of the oxide-bulk interface and the bulk layer or subsurface immediately below the interface will be referred to, for short, as the "surface properties."

It is an object of the present invention to provide a 50 method for producing semiconductor bodies with controlled surface, interface, subsurface, and oxide properties. This is accomplished by preferential oxidation of at least one of the principal components of a semiconductor alloy. During this process, impurities present in the system in trace amounts will also redistribute (see Atalla 2,953,486), but this is not the subject of this invention.

55 As is evident from the ensuing description, the present invention utilizes a forced oxidation, e.g. thermal and electrochemical oxidation, as distinguished from the spontaneous oxidation which some elements undergo in air under normal or room conditions, as for example aluminum or silicon. In such cases, the oxide coating forms until it reaches a characteristic thickness, after which further oxidation stops for all practical purposes. With SiGe alloys, spontaneous oxidation at room temperature nearly ceases at approximately 50 angstroms. The oxidation hereinafter disclosed provides much thicker oxidized metal coatings, for example, upwards of 200 angstroms. For most purposes, a will appear from the annexed drawings, coatings having thicknesses upwards from about 800 angstroms to as high as about 13,000 angstroms are produced in accordance herewith and will be found to be the most convenient and thus preferred. At these elevated levels of oxidation, rate limiting is not experienced before

the desired redistribution occurs to the significant extents that have been found to enable control of the characteristics of the semiconductor materials or devices formed in accordance herewith. At the low oxide coating thickness obtained with spontaneous oxidation, the oxide breakdown voltages are also too low for practical semiconductor devices.

#### Brief Statement of the Invention

The invention is based on the discovery of a number of surface changes which occur when alloys, as distinct from doped or undoped elemental bulk bodies, especially those alloys of Ge and Si, are oxidized; and on the realization that these changes may be utilized to facilitate processes and to produce products with improved performance as compared to known systems, especially those of Si and SiGe. The said discoveries may be summed up briefly as follows:

(1) On thermal oxidation of an alloy or composition of elements, e.g. SiGe, the bulk surface (oxide-bulk interface) and a bulk layer immediately thereunder are enriched in the less readily oxidized component, e.g. Ge in an SiGe alloy. The composition of the SiGe bulk layer of subsurface can be accurately adjusted in such a boundary layer.

(2) The oxide grown on the substrate upon a first oxidation consists predominantly of the oxide of the more readily oxidized element, e.g. in an SiGe alloy,  $\text{SiO}_2$  with a small Ge content not exceeding as a rule 1 atom percent, and Ge being present partly as elementary Ge and partly oxidized.

(3) By means of a number of operational cycles comprising each etching off a previously formed oxide coat and thermal oxidation, it is possible to arrive at an oxidized element coating which on an SiGe alloy is an  $\text{SiO}_2$  coating containing a proportion of Ge exceeding 1 atom percent, again partly as elementary Ge and partly oxidized, and this oxide has properties, such as growth-rate, etch-rate, and density, appreciably different from  $\text{SiO}_2$  or from oxide first grown on the same sample.

(4) Offset voltage, which is a measure of the oxide-bulk system, is less than for  $\text{SiO}_2$  on Si.

(5) Using oxidation to adjust the composition of semiconductor subsurface layers by selective oxidation is useful in other binary and ternary systems.

(6) Other oxidants including nitrogen and sulfur as well as other methods of achieving the oxidized state, e.g. electrochemical means, are contemplated for use with such binary and ternary systems, especially SiGe, to form the corresponding oxides, nitrides and sulfides.

#### Brief Description of the Drawings

In the following description reference will be had to the annexed drawings in which:

FIG. 1 is a diagrammatic representation of the volume changes in an oxidation-etching cycle.

FIG. 2 is a graphic representation of X-ray microprobe analysis of an oxidized SiGe alloy compared with an unoxidized control.

FIG. 3 is a graphic representation of the etching rates of  $\text{SiO}_2$  produced by a first oxidation on an Si and SiGe substrate.

FIG. 4 is a graphic representation of the MOS (metal-oxide-semiconductor) differential capacitance vs. voltage of a system according to the invention.

FIGS. 5 to 8 are graphic representations showing the mass change and accompanying changes in oxide thickness and etch-rate (in all but FIG. 6), on different SiGe alloys and different oxidation times on repeated oxidation-etching cycles.

FIG. 9 is a graphic representation of oxide thickness vs. time<sup>0.5</sup> for variety of different SiGe alloys and Si control after a first oxidation and a so-called steady-state oxidation.

FIG. 10 is a graphic representation of the thickness of the oxide layer vs. composition of SiGe alloys after one hour of oxidation for a first oxidation and for a so-called steady-rate oxidation.

FIG. 11 is a graphic representation of the etching rate of the oxide coat vs. composition of SiGe alloys for first and steady-state oxidation.

FIG. 12 is a graphic representation depicting the specific oxide mass (total mass/area) of a first and steady-state oxidation vs. time<sup>0.5</sup>.

FIG. 13 is a graphic representation showing the Ge pile-up as gradient profiles in the boundary layers at and below the interface and the Ge content in the oxide in a first oxidation and during three phases of a steady-state oxidation as time progresses.

FIG. 14 is a diagrammatic representation of one manner of application of the invention.

#### Detailed Description of Drawings and Invention

20 In FIG. 1  $M_1$  signifies the mass of an SiGe alloy prior to oxidation.  $M_2$  signifies the mass of the oxidized body (for simplicity only one surface is shown oxidized; in practice, all surfaces are oxidized unless shielded) and it is seen that the surface of the substrate which now forms the oxide-substrate interface has receded to below the original surface while at the same time the oxide layer has grown to project beyond that surface, the reason being that in the course of oxidation Si and Ge from the surface is converted into oxide.  $M_3$  in FIG. 1 signifies the residual substrate left after etching off of only the oxide layer from  $M_2$ .

In the following description the sequence of operations leading from  $M_1$  to  $M_3$ , i.e. oxidation of an etched substrate and etching off of the formed oxide layer will be referred to as one cycle. In one cycle  $M_1 - M_3$  signifies the weight loss in that cycle and  $M_2 - M_1$  signifies the weight gained during the oxidation phase of the cycle. There is defined as mass ratio

$$f = \frac{M_1 - M_3}{M_2 - M_1}$$

All masses are to be taken as specific masses, i.e. mass per  $\text{cm}^2$ .

It has been found in accordance with the present invention that while for oxidation of pure Si,  $f_{\text{Si}} < 1$ , for only a small removal of Ge from an SiGe sample,  $f_{\text{Ge}} > 1$ . This finding enables determination of the content of Ge in oxide coats grown on SiGe substrate. From the determination of the mass ratio  $f$  for various SiGe alloys and different oxidation times, the following conclusions were drawn:

- In an SiGe alloy, Si is oxidized in preference over Ge.
- The above preference is approximately independent of the compositions of the alloy and the time of oxidation, and a first oxide layer grown on an SiGe alloy contains Ge in an amount not exceeding 1 atom percent.

The experiments comprising oxidation, etching and weighing which led to the above and following observations were conducted as follows:

(1) Samples.—Two types of SiGe slices, each of 1.5-2  $\text{cm}^2$ , were used: polycrystals approximately (111) orientation heavily doped, 20-40 atom percent Ge, mainly for oxidation studies and single crystals up to 4.5 atom percent Ge, mainly for electronic studies.

Polycrystals were commercially produced thermoelectric material N and P having a resistance of approximately 0.001 ohm-cm., with large grains and twins (approximately 0.5 mm.), without cracks or voids, which etched and oxidized uniformly. They were solidified by the molten zone technique of Wang and Alexander (F. Rosi, Solid St. Elect., 11, 833 [1968] to obtain uniform ingot composition. In 10-15 atom percent Ge composition, composition varies less than 1% and boron doping,

on the order of 0.5%, along 10 cms. length (RCA 3rd Quarterly Report, SiGe Thermolectric Materials and Module Dev. Program July 1968-September 1968, ALO (2510)-3 AEC Res. & Dev. Report Cat. UC33, TID 4500). My electron microprobe X-ray fluorescence analysis of N-type samples indicated that the composition in selected small areas (approximately  $100\mu$  squares) of polished slices was uniform to better than 1% and phosphorus was uniformly distributed.

Single crystals were N and P 0.2-40 ohm-cm. grown in a conventional silicon crystal puller geared down to pull at rates of less than 2 cm./hour to minimize the effects of constitutional super-cooling. Crystals up to 9 cm in length were grown with shiny surfaces and 6 clearly defined facets. The bottom of each crystal was polycrystal resulting from melt enrichment. X-ray topograph of one slice of 3 atom percent Ge crystal showed regular annular striations like those encountered in heavily doped Si or Ge (J. A. M. Dikhoff, Phil. Tech. Rev. 25, 195 [1963]).

Composition of each slice was determined by density (J. Dismukes, J. Phys. Chem. 68, 3021 [1964]), resistivity by 4-point probe. Data are given in Table 1. Sawed samples were heavily etched and lapped and polished to remove damage. Final polish was diamond (0.25-0.5 $\mu$ ) on cloth. It should be noted that an initial etching step on a given sample may, in practice, be desired. The final step to produce an oxidized composite will, of course, be oxidation. To expose an enriched alloy surface, etching or removal of the oxidation product coating will be the final step.

TABLE 1.—SiGe SAMPLES

| Sample Number | Crystal | Atom percent Ge | Total area (cm. <sup>2</sup> ) | Thickness (microns) | Conductivity (ohm-cm.) | Type |
|---------------|---------|-----------------|--------------------------------|---------------------|------------------------|------|
| A             | Poly.   | 36.5            | 2.87                           | 356                 | 0.0021                 | N    |
| B             | do      | 36.5            | 3.41                           | 183                 | 0.0021                 | N    |
| C             | do      | 20.7            | 3.69                           | 243                 | 0.0017                 | P    |
| D             | Single  | 4.0             | 3.84                           | 257                 | 0.8                    | P    |

(2) Oxidation was done in a conventional horizontal wet oxygen system consisting of a partially closed tube at  $1063^\circ \pm 2^\circ$  C. Ambient-pressure oxygen was bubbled through deionized water at  $95^\circ$  C. Time was measured from time of insertion of sample in a small boat to time of withdrawal with no correction for warm-up for times of 25 minutes or more. Runs of 10 min. were accurately timed by inserting only the sample for fast warm-up using a long quartz vacuum-chuck. No effect on weight was found when samples were baked for 10 min. in dry oxygen at end of run.

(3) Oxide Etch was buffered HF (120 g.  $\text{NH}_4\text{F}$ , 43 cc. HF 48%, 250 cc. water) at  $22^\circ \pm 1^\circ$  C. agitated in a Teflon basket. Rate of etching of oxide on Si was found to be  $850-900^\circ$  A./min. To determine total time to remove oxide, the basket was lifted out of the liquid every 15 sec. Time was measured to that at which the sample floated when returned to the liquid since the sample is hydrophobic in contrast to the oxide. To be sure all oxide was removed, the sample was returned to the bath for one additional minute. The etched sample was then rinsed in deionized water, blotted dry and returned to the weighing chamber, whereby the cycle was completed. By weighing, it was verified that the etch bath etched the sample only to a negligible extent. However, the water was found to etch the sample about  $9\mu\text{g}/\text{min}$ , so rinsing was kept brief. "Sputtering" and other physical and chemical techniques may also be used to remove oxidized product coatings.

(4) Microbalance weighing was done with a Cahn Electrobalance Model 1500 using 1 mg. full-scale range. Precision is  $\pm 1\mu\text{g}$ , and reproducibility  $\pm 0.2\mu\text{g}$ . The balance setting shifts so little with time that overnight runs are possible. Sample is cleaned, balanced and balance time-stability checked. For maximum sensitivity,

the sample is made to weigh about 15 mg. which is the maximum weight allowed using the full beam of the balance. The sample itself is the pan and lightweight hangers of a few mg. weight are used. Thus with sample mounted, the beam is balanced to zero ( $M_1=0$ ) and calibrated to full-scale with the 1 mg. weight. These settings are checked and then locked. After oxidation, the sample is weighed ( $M_2$ ). After etching off the oxide, the sample plus the 1 mg. calibrating weight is weighed (1 mg.— $M_3$ ), ending the weighing cycle.

(5) Thickness was measured by conventional interferometric technique using evaporated Al over the etched oxide-to-sample step. Good agreement was found (see discussion of FIG. 3) when thickness was also determined by  $\text{SiO}_2$  interference colors (W. A. Pliskin and E. E. Conrad, IBM J. Res. Develop. 8, 43 [1964]), so color was used in most cases. An important first experiment was done which showed (Table 2) that the doping impurity did not appreciably interfere with the composition effect being studied. In Table 2 an increase in thickness is shown of about 10 A./atom percent Ge for oxide grown on a fresh surface.

TABLE 2.—FOUR-HOUR FIRST OXIDATION

|                      | Ohm-cm. | Oxide color | Color thickness, A. |
|----------------------|---------|-------------|---------------------|
| Silicon              | 0.01    | N           | Violet              |
| 4.3 atom percent Ge  | 0.22    | P           | Blue violet         |
| 36.5 atom percent Ge | 0.0012  | P           | Green               |
| 36.5 atom percent Ge | 0.0021  | N           | do                  |

(6) Ge Surface pile-up was measured directly by use of the Jeolco electron microprobe analyzer measuring the Ge  $\text{L}\alpha$  X-ray line at 5.5, 10 and 25 kv. in order to penetrate to different depths. An unoxidized control was compared to an oxidized adjacent piece of the same sample.

(7) Oxide electrical properties were measured on the Boonton 75C capacitance bridge and the Boonton 71A capacitance meter.

(8) Oxide infrared transmission was measured on the Perkin-Elmer Model 21 double-beam spectrometer in the vicinity of 9 and 12 microns comparing an oxidized sample to a matched sample without oxide.

The expression "first oxidation" used hereinbefore and to be used hereinafter refers to the oxidation of a surface on which there are no traces of any previous appreciable oxidation history. Consequently, for a first oxidation it is always necessary to first etch the surface of the substrate down to a depth sufficient to remove completely any oxide layer and sufficient layer of the bulk that may have been affected by previous appreciable oxidation (see, for example, discussion of FIG. 5).

The presence of Ge in a first oxide layer grown at  $1065^\circ$  C. on a polycrystal SiGe sample of 14 atom percent Ge was determined by infrared absorption measurement, which showed a slight shift in the direction that was to be expected from Ge. The sample was run together with a matched unoxidized SiGe blank. Pure Si was oxidized and run in a double-beam spectrometer, similarly against a matched blank. Comparing the two, peaks shifted from approximately  $9.25\mu$  ( $\text{SiO}_2$ ) to  $9.4\mu$ , and from  $12.3\mu$  ( $\text{SiO}_2$ ) to  $12.6\mu$ .

Together with the preferential oxidation of Si from an SiGe alloy there occurs a Ge pile-up at the interface and in the bulk layer immediately below the interface. This pile-up was determined by an X-ray microprobe surface analysis of a 36.5 atom percent Ge P-type sample after

first oxidation. This sample was scribed and broken into two parts one of which was oxidized to a thickness of 5200 Å. and oxide removed. The two pieces were mounted side by side and X-ray fluorescence counting of Ge L $\alpha$  line was done at several points on both pieces. (It is interesting that, comparing the two pieces, the unoxidized control looked "darker." That is, the effect of Ge enrichment of the surface was visible with the unaided eye.) Counts, after small background correction and small beam current normalization, were compared at 5.5, 10 and 25 kv.

The data are shown in Table 3 together with an estimate of depth that is sampled by the beam. Depth estimate was obtained from measurements of depth in Cu from which 95% of X-ray yield came (U. Schmitz, P. L. Ryder, W. Pitsch, 5th Intl. Cong. X-Ray Optics & Microanalysis, Tubingen [1969], p. 104). By use of the electron range relation (V. E. Coslett and W. C. Nixon, "X-Ray Microscopy," Cambridge [1960], p. 223)

$$X_R = \frac{A}{\rho z} V^2$$

$$X_R = aA/\rho_z V^2$$

where A=atomic weight,  $\rho$ =density, z=atomic number V=accelerating voltage, and  $a$ =constant, one obtains from the Cu data at 20 kv. for Si  $X_R = 3.3 \mu$  and for

$$GeX_R = 1.7 \mu$$

For the compositions 36.5 atom percent Ge and using the  $V^2$  dependence of electron range relation, the depth estimates of Table 3 are obtained.

TABLE 3.—SURFACE Ge L $\alpha$  X-RAY DATA

| V (kv.)     | Average counts (10 sec.) | Back-ground (10 sec.) | Beam current (ma.) | Relative intensity | Estimated range ( $\mu$ ) |
|-------------|--------------------------|-----------------------|--------------------|--------------------|---------------------------|
| 5.5 sample  | 7,017                    |                       | 34                 | 1.64               | 0.2                       |
| 5.5 control | 4,557                    | 107                   | 36                 | 1                  |                           |
| 10 sample   | 19,161                   |                       | 44                 | 1.36               | 0.7                       |
| 10 control  | 14,668                   | 211                   | 46                 | 1                  |                           |
| 25 sample   | 39,416                   |                       | 45                 | 1.15               | 4.2                       |
| 25 control  | 34,287                   | 2,596                 | 45                 | 1                  |                           |

The results of the above measurements are shown graphically in FIG. 2 in which the relative X-ray yield is plotted against the range, i.e. depth below the surface (oxide-bulk interface). As is shown, there is a strong pile-up of Ge of the order of 2. It is further seen from FIG. 2 that toward the interior of the bulk body the Ge concentration approaches gradually that of the Ge content in the unoxidized sample. This level of Ge concentration is reached practically already at a depth of 4 $\mu$ .

Since the oxide layer grown by a first oxidation on an SiGe alloy consists predominantly of SiO<sub>2</sub>, it was to be expected that the rate of its etching off should be similar to that of SiO<sub>2</sub> grown on pure Si. This was confirmed experimentally as shown in FIG. 3 where the thickness of oxide grown on pure Si and on an SiGe alloy containing 36.5 atom percent Ge, both at 1063° C. for one hour in wet oxygen, is plotted against etching time in minutes. Initial and final thickness was measured interferometrically on an aluminized step. Intermediate thickness was measured by SiO<sub>2</sub> interference color. The Si control was oxidized alongside the sample in the same boat and this control oxide showed a slightly different color. This color difference persisted as sample and control were etched together which indicates that the etching rate of the first oxide of both the control and the sample were the same. The color difference was checked at  $t=50$  minutes by aluminizing the step and measuring the interference fringe displacement. Agreement in the color difference at both times means that the index of refraction of the first oxide was close to that of SiO<sub>2</sub>.

An important difference in first oxide grown on SiGe as compared to Si control was discovered by MOS capacitance measurements. Measurements were conducted on a system comprising an evaporated aluminum counter-electrode applied to an approximately 2200 Å. first oxide

grown on an 0.2 ohm-cm. N-type SiGe alloy of 2.5 atom percent Ge content. The results of the measurement are shown in FIG. 4 where capacitance is plotted against voltage and it is seen that the first oxide gives a flat-band voltage of approximately 0 as compared to -4 to -6 v. obtained with 2200 Å. of SiO<sub>2</sub> grown by the same process on pure Si.

The mass changes occurring during several cycles of 10 minutes oxidation are diagrammatically illustrated in FIG. 5. Part (a) of FIG. 5 plots  $M_2 - M_1$  and  $M_1 - M_3$  (see FIG. 1) as a function of the number of oxidation/etch cycles. In Part (b) of FIG. 5 the lower curve plots the oxide color thickness (left-hand side ordinate) as a function of the number of cycles, and the upper curve plots the oxide removal time by etching (right-hand side ordinate) as a function of the number of cycles. Cycles 1a, 1b, and 1c of FIG. 5 are considered each as first oxidation since in each case after the weight cycle, i.e., after  $M_3$  was measured, a layer of 4 microns, i.e.  $4 \times 10^4$  Å. or more was etched off. Oxide thickness in this as well as other tests herein set forth was determined by SiO<sub>2</sub> color and etch removal time in same cycles. Indeed it is seen from FIG. 5  $M_1 - M_3$ ,  $M_2 - M_1$ , oxide layer thickness and oxide layer removal time for these three cycles are about 20 the same, which confirms the assumption that each of these cycles may be considered as a first oxidation.

From the values in Part (a) of FIG. 5 the mass ratio  $f$  for each cycle can be calculated by comparing them with known ratios for an oxide grown on pure Si, it may 30 be concluded that the first oxide grown is nearly pure

SiO<sub>2</sub> and that consequently the sample surface must be enriched with Ge after oxidation.

After cycle 1c only the oxide layer is etched off and the remaining sample is reoxidized. In this case the oxidation is no longer a first oxidation. In the then following cycles the same procedure is followed, i.e. the oxide alone is etched off and the remaining sample is reoxidized. From the  $M_1 - M_3$  and  $M_2 - M_1$  curves of Part (a) of FIG. 5 it is seen that in these cycles a profound change 50 occurs as compared to the first oxidation cycles 1a, 1b and 1c. This is seen most strikingly with thin oxide colors. The sample oxidizes first to gold yellow (with a touch of rose pink) about the same on all grains. In cycle 2 under the same conditions there is obtained a rich blue and the 55 etch time of the oxide of this cycle almost doubles. In subsequent cycles color and etch time change only slightly. However, in cycles 2, 3, 4 and 5 the surface of the sample progressively loses its polish in some areas. That is, after cycle 2 the center of the sample surface appears a 60 bit roughened as though stained. Patches of texture appear which do not follow grain structure. Under high magnification patches are seen to contain shallow pits. After cycle 3 the surface is about 20% matte and after cycle 4 about 40%.

The same sample was oxidized and etched in cycles of 4 hour oxidation and the results are shown in FIG. 6. Again, first oxidation of newly polished and etched surface gives a mass ratio like SiO<sub>2</sub>. Subsequent cycles show great variations in mass of sample consumed, but not much variation in oxygen taken up. One month elapsed between 70 cycles 6 and 7 as compared to a period of the order of 1 day between other cycles.

A sample of an SiGe alloy containing 36.5 atom percent Ge (sample B—Table 1) was oxidized and etched in cycles 75 of 40 minutes oxidation and the results are shown in FIG.

7. Data  $M_1 - M_3$ , sample consumed, are like FIG. 6 for cycles 3-7, suggesting variations around a steady value. Cycles 8 and 9 show increased  $M_1 - M_3$  in each cycle like FIG. 5. Oscillation in  $M_2 - M_1$  data is clearly seen with complementary oscillation in  $M_1 - M_3$  data. This suggests weight loss due to evaporation of Ge is affecting the data. This sample oxide was violet-purple after cycle 1 but mottled purple to jade green after cycle 2. First oxide was like polished Si. Second oxide had little dark regions on the sample surface which were present before and after oxide was removed. Cycle 3 caused the sample to appear more uniformly matte before and after oxide was removed. This uniform matte surface persisted subsequently.

FIG. 8 shows the results of the oxidation of a sample of composition 20.7 atom percent Ge (sample C, Table 1) in cycles of 40 minutes oxidation time. Mass of oxygen taken up per unit area by the sample surface is roughly the same as shown in FIG. 7 (for sample with 36.5 atom percent Ge for 40 minutes), but comparing cycles 3 through 8, mass of sample consumed is somewhat less. This suggests that after first oxidation a monotonic dependence on composition exists.

On the basis of the raw weighing data represented in FIGS. 5 to 8, a distinction is made between a first oxidation and oxidation cycles 3, 4, 5, etc., which has been referred to and will be referred to hereinafter as steady-state oxidation.

In FIG. 9 the thickness of the oxide layer is plotted against the time<sup>0.5</sup> for various samples including pure Si and for first (1) and steady-state (S) oxidation. The solid line in FIG. 9 joins points for pure Si. It is seen by the pair of points at 25 minutes that the first oxide of sample D of Table 1-4 atom percent Ge—is approximately 100 Å. thicker than oxide on Si, and first oxide thickness increases about 10 Å./atom percent Ge (see Table 2).

In FIG. 10 the thickness of the oxide layer after oxidation for one hour is plotted against the Ge content in the SiGe substrate for first (1) and steady-state (S) oxidation and it is seen that even a low Ge content induces a small extra oxide thickness.

Etch-rate vs. SiGe substrate composition for first and steady-state oxidation is plotted in FIG. 11. At 4 atom percent Ge, etch-rate of the first oxide is approximately that of  $\text{SiO}_2$ . At 20-36.5 atom percent Ge, etch rate of the first oxide is approximately 85%, and of the steady-state oxide 57%, of the  $\text{SiO}_2$  rate and independent of sample composition. Buffered HF etch is carried out at approximately 22° C. (10-minute first oxidation does not seem to be consistent with longer time. This may indicate excess Ge.)

In FIG. 12 the total mass/area of first oxides and steady-state oxides are plotted against time<sup>0.5</sup> for samples A and B of Table 1. The result for the first oxidation (lower curve) agrees closely with published values for growth of oxide on pure Si (solid line) which is surprising. It means that Ge at the growing oxide/SiGe interface does not appreciably impede the growth of  $\text{SiO}_2$ . Against this, the results for steady-state oxidation differ from those for  $\text{SiO}_2$  and this is discussed further below.

Some of the mass ratio,  $f$ , from the first oxidation data in FIGS. 5 to 8 are 0.889 as compared to 0.8775 for pure  $\text{SiO}_2$ . Some deviate from this presumably because of weight loss caused by evaporation of  $\text{GeO}_2$ . It is, however, important to realize that the total mass of oxide,  $M_2 - M_3$ , is measured (FIG. 12) independently of weight loss from the system and first oxide agrees closely with  $\text{SiO}_2$  data.

By referring once again to FIGS. 5 to 8 it is seen that the weighing data after first cycle shows lower observed oxygen up-take ( $M_2 - M_1$ ) than first oxidation and a much larger sample consumption ( $M_1 - M_3$ ). Large variations in mass are evident but average values may be considered for the purpose of analysis.

Steady-state oxide grows thicker than first oxide in one hour. As shown in FIG. 10, the thickness of oxide in one hour in the limit of a few percent Ge in the bulk is about

6000 Å., about 11% greater than on pure Si, and it increases about 20 Å./atom percent Ge. That is, most of the extra thickness of steady-state oxide is found even at low concentrations. The rate is relatively insensitive to more Ge thereafter, much like first oxide. However, after 16 hours, oxide thickness is close to that expected for  $\text{SiO}_2$  on Si.

Etch-rate is markedly lower on steady-state oxide (FIG. 11) grown 10 minutes to 1 hour, dropping to about 57% of  $\text{SiO}_2$  rate, independent of bulk composition between 20-40 atom percent Ge. However, for thick oxide, grown 16 hours, etch rate is like  $\text{SiO}_2$  rate.

Thickness by color is in good agreement with step-height measurements, i.e. index of refraction is not sensitive to oxide composition.

Total specific mass ( $M_2 - M_3$ ) of steady-state oxide vs. time<sup>0.5</sup> of FIG. 12 is seen to be more massive when compared to specific mass of first oxide at one hour. The excess mass appears to be decreasing with time, being less large at four hours. Since, after 16 hours oxidation compared to Si control, oxide thickness and oxide etch rate are nearly the same, it is concluded that excess mass is a small percent of total oxide mass after 16 hours. By comparing excess mass from the upper curve of FIG. 12 and excess thickness from FIG. 9 after one hour, density of oxide relative to  $\text{SiO}_2$  can be obtained.

Thus mass, thickness and etch rate suggest that initial excess of substrate Ge is incorporated into the growing oxide. Presumably this occurs because of piled up Ge which remains after first oxidation. After about two cycles an approximate steady-state is reached in which Ge is incorporated during the first time of oxidation. This effect is diluted out by continued long-time oxidation which then becomes much like first oxidation. Since the effect occurs early, it is sensitive to initial surface conditions before each oxidation. This accounts for the large variation in sample up-take. It should be noted that oxygen up-take does not show large variation (FIG. 6) which indicates that Ge is incorporated into the oxide without oxygen.

The distinction between a first oxidation and the steady-state oxidation is diagrammatically represented in FIG. 13. Part (a) of FIG. 13 represents a first oxidation while Parts (b), (c) and (d) of FIG. 13 represent three phases during a steady-state oxidation, Part (b) approximately 1 minute, Part (c) approximately after 40 minutes, and Part (d) approximately after 4 hours. Solid curves are Ge concentration plotted against distance in oxide layer and in SiGe substrate. Vertical solid lines mark the gas/oxide and oxide/substrate interfaces in each of FIGS. 13b, 13c and 13d as in 13a.

Referring to Part (a) it is seen that in the SiGe bulk there is a pile-up or increase in concentration of Ge toward the interface which reaches its maximum value at the interface. In the oxide layer there is a small Ge content of the order of 1 atom percent which drops along a concentration gradient profile toward the oxide surface. It is considered that the Ge in the oxide layer is predominantly in the form of elementary Ge and not oxidized.

At the initial phase of steady-state oxidation, depicted in Part (b) of FIG. 13, an initial transient occurs because of Ge surface enrichment resulting from previous oxidation. During this transient, excess Ge is incorporated in the growing oxide, some  $\text{GeO}_2$  evaporates, and other transient effects may occur resulting in pitting. As the oxide layer grows in thickness (Parts (c) and (d)), the Ge content and Ge distribution in surface and oxide changes and approaches the same gradient profile as in a first oxidation.

Based on all the above observations and conclusions, the invention in its broadest aspects consists in a process for producing from a semiconductive alloy, e.g. an SiGe alloy, a composite body having a controlled coating comprising mainly the oxidation product of the more easily oxidized element of the alloy and a controlled pile-up at

## 11

the oxide-bulk interface of the element less readily oxidized in the boundary layer, wherein the substrate is subjected to an oxidizing atmosphere. Preferably, the exposure is to an oxygen-containing atmosphere at an elevated temperature within the range of 700-1300° C. The oxidation step may be preceded by or the process terminated by an etching step to remove oxidized element from the surface of the composite body. The invention also is in the products produced by the process and in its use as a fabrication technique or as an intermediate step in semiconductor processing.

In accordance with one embodiment of the invention, the substrate is subjected to one single etch/oxidation cycle, thereby producing a composite body with an oxide coat containing Ge in an amount not exceeding 1 atom percent.

In accordance with another embodiment of the invention, the substrate is subjected to more than one of said cycles to produce an oxide coat containing an increased proportion of Ge, usually more than 1 atom percent Ge, the etching after each oxidation being so designed as to remove essentially only the oxide coat formed in the previous cycle except in the last step in which the oxide coat may be retained. The number of cycles may be from 1 to 10 or more, if desired. The number of cycles, the temperature, and other parameters of oxidation, e.g. time, will be determined by the final concentration of Ge desired in the oxide coating or at the surface of the bulk material. After a number of cycles for a given alloy, further oxidation/etch cycles do not confer such a material change in Ge concentration that further cycling is beneficial.

If desired, it is possible in accordance with the invention to etch off the oxide coat produced by oxidation after the last cycle to produce a product with no oxide coat and having a predetermined Ge pile-up at the surface; such a product can be used for further processing in any desired way.

While the invention has been exemplified with a specific class of alloys and oxygen or water vapor as the oxidant material, it will be understood that the principles of this invention may be applied to other binary and ternary alloy bulk bodies. Instead of oxygen, other oxidants for the differentially oxidizable alloy moieties may be used in partial or total replacement for the oxygen, e.g. sulfur, nitrogen, etc., to form the sulfides or nitrides as a coating on the bulk material. Other oxidation processes, such as anodic oxidation, may be employed.

By means of the method according to the invention, it is possible to achieve, among others, the following advantages in the semiconductor field:

- (1) Improved MOST (metal oxide semiconductor transistor) devices because of lower or controllable offset voltage, higher lateral surface mobility (at high Ge concentration), higher transconductance, and better oxide;
- (2) Improved bipolar devices, for example, lower non-ideal surface current and reduced base resistance;
- (3) New-type resistors, capacitors and other passive elements, e.g. improved MOS capacitors by control of flat-band voltage, conductance, specific capacitance;
- (4) More reliable devices whose Ge-containing oxide coat is more dense and possibly less permeable than pure  $\text{SiO}_2$ ;
- (5) New metal semiconductors or Schottky-barrier devices;
- (6) SiGe heterojunction devices fabricated with advantages in photo-absorption and as wide-narrow gap diode, as for example, wide-gap emitter;
- (7) Lateral transistors improved by more favorable lateral injection into Ge-rich surface base-layer;
- (8) Improved photodevices taking advantage of differing energy-gap in the subsurface relative to the bulk body.

## 12

One embodiment of a semiconductor product produced in accordance with the invention is shown diagrammatically and by way of example only in FIG. 14. In that figure a substrate 1 is shown consisting of an Si or SiGe base on which a thin layer of an SiGe alloy is grown epitaxially, which layer constitutes the substrate for oxidation in accordance with the invention. Discrete circular zones 2 are defined by adequately masking the substrate, and oxidized. The structure of each oxidized zone 2 is shown in the upper part of FIG. 14. It comprises a Ge-rich layer 3 in which there is a Ge pile-up, e.g. as in FIG. 13, and an oxide coat 4 of a desired Ge content, depending on whether the coat was produced by one- or multi-cycle oxidation. The substrate below layer 3 is not shown in the upper part of FIG. 14; it is the same as prior to oxidation.

Other devices and integrated circuit fabrication processes which are contemplated by this invention are:

(a) Selective use of alloy and oxide for selective oxidation, selective etch-down to make configurations, selective masking of some regions of substrate Si relative to other regions, controlled by variations in oxide properties,

(b) Control of properties over a semiconductor surface by pre-depositing alloy and oxidizing as described above,

(c) Inserting Ge-rich regions by this process to utilize properties such as different mobility, energy gap, ionization coefficients, thermal conductivity, stress-moduli, potential barrier-heights in metal-semiconductor configurations, dielectric constant,

(d) Method of fabricating Ge-Si or near Ge-Si heterojunction,

(e) Use of layers from the process to advantage in ion implantation,

(f) Take advantage of different properties of impurities in Ge-rich region resulting from the process, relative to other regions; different properties being for example diffusion rates, solubilities, segregation, and energy levels of impurities, wetting and alloying, and contacting properties,

(g) Use surface layer or oxidation as an intermediate step in fabrication, not necessarily retained in completed device,

(h) Control of surface potential and/or interface-state densities in oxidized devices and integrated circuits,

(i) Use of multiple layers by combining epitaxial deposition of alloy with this process, for example to make a sandwich of  $\text{SiO}_2/\text{Ge}/\text{Si}$ ,

(j) Oxidize SiGe on Ge in order to form  $\text{SiO}_2$  thermally on Ge,

(k) Use deposited (not thermally grown)  $\text{SiO}_2$  in regions where Ge pile-up is not desired in this process,

(l) Use anneal post-treatment to advantage.

What is claimed is:

1. A process for producing a composite body from a bulk body of a silicon/germanium alloy containing more than 1 atom percent germanium, said body being characterized by (a) a coating comprising silicon dioxide, (b) an interface between the silicon dioxide-containing coating and the bulk body and (c) a boundary layer contiguous to said interface having an increased concentration of germanium therein; comprising the step of oxidizing the bulk body with an oxidant for silicon.

2. A process in accordance with claim 1 wherein the silicon dioxide coating has a thickness greater than 200 Å.

3. A process in accordance with claim 1 wherein the silicon dioxide coating has a thickness greater than 800 Å.

4. A process in accordance with claim 1 wherein the silicon dioxide coating has a thickness between 800 and 13,000 Å.

5. A process in accordance with claim 1 in which the temperature range for the oxidation step is from 700° C. to 1300° C.

13

6. A process in accordance with claim 5 in which the silicon/germanium alloy is first epitaxially deposited on a silicon base.

7. A process in accordance with claim 1 which is additionally characterized by the step of etching the surface with an acid reactive only with the silicon dioxide coating alternately performed with said step of contacting with an oxidizing agent.

8. A process in accordance with claim 7 in which the steps of removing the silicon dioxide coating and oxidizing the bulk surface are repeated until steady-state oxidation is achieved.

9. A process in accordance with claim 1 wherein the process consists essentially of the steps of (a) etching the surface with an acid reactive with  $\text{SiO}_2$  and (b) oxidizing the etched surface with an oxygen-containing gas at a temperature in the range of from 700° C. to 1300° C. to yield an  $\text{SiO}_2$  coating thereon, the boundary layer being enriched in germanium.

10. A process in accordance with claim 7 in which the semiconductive alloy consists of from about 4 atom percent to 37.5 atom percent of germanium, balance silicon, the oxidant is oxygen, and the reactive acid is a dilute or buffered aqueous solution of hydrogen fluoride.

11. A process in accordance with claim 1 in which the terminal step is etching to remove all traces of  $\text{SiO}_2$ .

12. A process for producing a composite body from a bulk body of a silicon/germanium alloy containing >1

14

atom percent germanium, said body being characterized by a boundary layer in which the concentration of the germanium is in excess of the concentration of the germanium in the bulk body comprising the steps, alternately performed, of (a) contacting the bulk body with an oxidant for the silicon at a temperature in the range of from 700° C. to 1300° C., to form a coating of the oxidation product on said bulk body, and (b) removing the oxidation product coating from the surface with an acid reactive only with the oxidation product coating.

13. A process in accordance with claim 12 in which the final step is oxidation.

14. A process in accordance with claim 12 in which the final step is removing the silicon dioxide coating.

15 References Cited

UNITED STATES PATENTS

|           |         |                 |       |            |
|-----------|---------|-----------------|-------|------------|
| 3,287,162 | 11/1966 | Chu             | ----- | 317—235 AG |
| 3,441,812 | 4/1969  | Bucs et al.     | ----- | 317—235 AG |
| 3,398,029 | 8/1968  | Yasufuku et al. | ----- | 317—235 AG |
| 3,342,567 | 9/1967  | Dingwall        | ----- | 317—235 AP |

ALFRED L. LEAVITT, Primary Examiner

M. F. ESPOSITO, Assistant Examiner

U.S. CL. X.R.

117—201, 118; 75—134 G, 134 S; 317—235 AG, 235 AP